

Patented May 14, 1929.

1,712,621

# UNITED STATES PATENT OFFICE.

CHARLES S. JOHNSON, OF CHAMPAIGN, ILLINOIS.

## METHOD FOR DETERMINING THE MOISTURE CONTENT IN AGGREGATES.

No Drawing.

Application filed March 12, 1927. Serial No. 175,011.

This invention relates generally to the art of making concrete, and more particularly to a method for determining the amount of moisture in aggregates having a variable moisture content.

It is well recognized that the strength of concrete depends largely upon the total water in the mix and that variations in the total water content cause unknown and undesirable variations in the strength of the concrete. For this reason, to obtain concrete of uniform and predetermined strength, it is necessary to determine accurately the total amount of water in each mix.

Commercial building aggregates such as sand, gravel, etc., have a variable moisture content which not only affects the apparent volumes of a quantity of aggregates of a given dry-aggregate-content, but also affects the total water in the mix when the water and aggregates are proportioned independently of each other by volume or by weight, and then combined. Thus if a specified quantity of water is combined with quantities of aggregates of variable moisture content which have been proportioned either by volume or by weight, the moisture in the aggregates is added to the water and thereby increases the total water in the mix to an unknown quantity.

It is the general object of the invention to provide a method whereby the moisture content of aggregates may be readily and accurately determined, thereby to permit an operator to hold the total water in the mix constant by combining with the separately proportioned bulk aggregates a quantity of water such that the sum of the moisture content of the aggregates as determined by this method and that of the water added independently, equals a predetermined specified amount.

Another object is to provide such a process for determining the moisture content of commercial building aggregates of variable moisture content which lends itself readily to practical use and field application.

Other objects and advantages will become apparent as the description proceeds.

It has been found as a result of a large number of experiments, that the specific gravity of building aggregates is remarkably constant even when these aggregates are

obtained from widely separated sources. As the specific gravity of the aggregate, i. e., the specific gravity of the dry-aggregate-content, remains unaffected by variations in moisture content, I utilize this characteristic as a basis for my invention.

The invention contemplates a process whereby a sample of an aggregate is first weighed in air and is then weighed suspended in water, provision being made so that when the sample is weighed suspended in water the moisture already in the sample is permitted to combine with the water. The weight of the moisture in the original sample is thereby automatically subtracted from the weight of the solid material so that the weight of the sample suspended in water indicates the weight of the dry-aggregate-content of the original sample. Knowing the specific gravities of the aggregate and of the water, the moisture content of the original sample may then be readily determined.

For the purpose of more fully describing the invention I shall, for an example, assume that commercial building aggregates have a specific gravity of 2.7, that water weighs 62.5 pounds per cubic foot and has a specific gravity of 1.0, and that a sample of bulk aggregate is selected which weighs 17 pounds in air. If this sample contains only absolutely dry aggregate, i. e., aggregate having no moisture content, its weight suspended in water will equal the weight in air minus the loss in weight when submerged in water,

$$\text{or } (\text{weight in air}) - \frac{(\text{weight in air})}{2.7 \times 62.5} \times 62.5 \quad 90$$

$$\text{or } 17 - \frac{17}{2.7},$$

$$\text{or } 17 - 6.3,$$

$$\text{or } 10.7 \text{ pounds.} \quad 95$$

If a sample containing moisture is weighed in air, it will be apparent that when that sample is weighed submerged in water the loss in weight will be greater than 6.3 pounds because the moisture contained in the original sample combines with the water automatically so that only the dry-aggregate-content of the sample is effective in displacing water. If, for example, the weight of the sample in air is 17 pounds as before, and its weight when submerged in water is 10 pounds, the

original sample contained 10.7-10, or .7 pound of moisture. This is equal to

$$\frac{.7}{17} \times 100 \text{ or } 4.12\%$$

moisture content, for the increased loss in weight of the sample when weighed submerged in water must have been due to the automatic subtraction of the weight of the moisture in the sample which combined with the water.

Thus by weighing a sample of normally moist aggregate in air and then weighing the same sample submerged in water so that the moisture in the aggregate has combined with the water, the weight of the dry-aggregate-content of the sample under water is determined. By then comparing this dry-aggregate-content weight of the sample with the known or theoretical weight in water of a mass of dry sand which has a weight in air equal to the weight in air of the sample, it is possible to determine the moisture content of the sample. The weighing of samples of the

aggregates in air, and then weighing them 25 submerged in water, constitutes a simple process by which the moisture content may be readily determined.

I claim as my invention:

1. As a step in the preparation of concrete, 30 the process of determining the moisture content of aggregates of variable moisture content which includes weighing a quantity of an aggregate in air, placing said quantity in water so that the moisture in the aggregate 35 combines with the water and then weighing the dry-aggregate-content of said quantity.

2. A process of determining the moisture content of aggregates which includes weighing a quantity of a normally moist aggregate 40 in air, placing said aggregate in water so that the normal moisture thereof combines with the water and then weighing the dry-aggregate-content of said quantity submerged in water.

In testimony whereof, I hereunto affixed my signature.

CHARLES S. JOHNSON